# EUROPEAN PATENT SPECIFICATION

(11) **EP 3 246 426 B1**
(45) Date of publication and mention of the grant of the patent: **24.06.2020**
(21) Application number: 16737217.6
(22) Date of filing: 15.01.2016
(51) Int. Cl.: C21D 9/46, C22C 38/02, C22C 38/04, C22C 38/06, C22C 38/08, C22C 38/12, C22C 38/16, C22C 38/42, C22C 38/44, C22C 38/46, C22C 38/48, C22C 38/50, C22C 38/54, C22C 38/00, C22C 38/58, C21D 6/00, C21D 8/02, B21B 3/00, B21B 1/02, B21B 3/02, C21D 9/00, C21D 7/13

(54) **METHOD FOR MANUFACTURING A THICK HIGH-TOUGHNESS HIGH-STRENGTH STEEL SHEET**
VERFAHREN ZUR HERSTELLUNG VON EINEM DICKEN HOCHROBUSTEN HOCHFESTEN STAHLBLECH
PROCÉDÉ DE FABRICATION D'UNE TÔLE D'ACIER ÉPAISSE DE HAUTE TÉNACITÉ ET DE HAUTE RÉSISTANCE

(30) Priority: 16.01.2015 JP 2015006670
(43) Date of publication of application: 22.11.2017
(73) Proprietor: JFE Steel Corporation, Tokyo 100-0011 (JP)
(72) Inventor: KITSUYA, Shigeki, Tokyo 100-0011 (JP); ICHIMIYA, Katsuyuki, Tokyo 100-0011 (JP); HASE, Kazukuni, Tokyo 100-0011 (JP)
(74) Representative: Grünecker Patent- und Rechtsanwälte PartG mbB
(86) International application number: PCT/JP2016/000197
(87) International publication number: WO 2016/114146

(56) References cited:
- EP-A1- 2 765 210
- EP-A1- 3 120 941
- EP-A1- 3 135 787
- EP-A1- 3 222 744
- WO-A1-2014/141697
- WO-A1-2015/140846
- WO-A1-2015/162939
- CN-A- 101 962 741
- CN-A- 102 605 280
- JP-A- H04 285 119
- JP-A- H07 232 201
- JP-A- 2002 210 502
- JP-A- 2002 256 380
- JP-A- 2011 153 366
- JP-A- 2011 202 214
- JP-B1- 5 590 271
- JP-B1- 5 598 618
- JP-B2- 3 333 619

## Description

### Technical Field

The present invention relates to a method for manufacturing a thick-walled high-toughness high-strength steel plate for use in steel structures in construction, bridges, shipbuilding, offshore structures, construction and industrial machinery, tanks, penstocks, and the like. In particular, the surface of the steel plate has high toughness, and the inner part of the steel plate has high strength and toughness. The steel plate has a thickness of 100 mm or more and a yield strength of 620 MPa or more.

### Background Art

In general, steel for use in construction, bridges, shipbuilding, offshore structures, construction and industrial machinery, tanks, penstocks, and other fields is welded to have a desired shape. In recent years, with significantly increasing in size of steel structures, the strength and thickness of steel to be used have also been greatly increased.

Despite trying to manufacture a thick-walled high-strength steel plate having a thickness of 100 mm or more and having high strength and toughness in a half-thickness portion (the central portion in the thickness direction), a structure having relatively low strength, such as ferrite, tends to be formed in the half-thickness portion due to a decreased cooling rate. Thus, the addition of large amounts of alloying elements is required to reduce the formation of such a structure.

In particular, in order to achieve high strength and toughness of a half-thickness portion of a thick-walled material (a thick-walled steel plate having a thickness of 100 mm or more), it is important to form bainite or a mixed structure of bainite and martensite in the half-thickness portion during quenching. This requires the addition of large amounts of alloying elements, such as Mn, Ni, Cr, and/or Mo.

The cooling rate is higher on the surface of a steel plate than in the half-thickness portion. Thus, a martensite structure having low toughness is formed on the surface of the steel plate. Thus, a high-strength steel plate having a thickness of 100 mm or more rarely has both high surface toughness and high strength and toughness of the inner part thereof.

A steel plate related to the present invention is described in the following two pieces of non-patent literature, for example. Non Patent Literature 1 describes a material having a thickness of 210 mm, and Non Patent Literature 2 describes a material having a thickness of 180 mm.

CN 102605280 A describes a method for manufacturing an ultra-thick high-strength high low-temperature toughness steel plate for ocean platforms, wherein the steel plate comprises, in weight percentage, 0.10-0.24% of C, 0.05-0.35% of Si, 0.60-1.15% of Mn, not more than 0.015% of P, not more than 0.005% of S, 0.01-0.030% of Ti, 1.45-1.75% of Cr, 0.15-0.44% of Mo, 0.80-2.50% of Ni, 0.010-0.070% of Nb, 0.020-0.080% of V, 0.02-0.06% of Alt, 0.001-0.004% of Ca, not more than 0.006% of N, 0.0007-0.0030% of B, the balance being Fe and unavoidable impurities and whereing the steel plate has a system of C, Ni-Cr-Mo alloyed and Nb-V-Ti microalloyed, and has a yield strength not smaller than 690MPa, a tensile strength not smaller than 770MPa, -40°C Charpy V-notch impact energy not smaller than 69J, NDT (non-destructive testing) not larger than -35°C, Z not smaller than 35%, and largest thickness of more than 200mm.

### Citation List

### Non Patent Literature

NPL 1: Nippon Steel Technical Report, 348 (1993), 10-16
NPL 2: Nippon Kokan Technical Report, 107 (1985), 21-30

### Summary of Invention

### Technical Problem

These pieces of non-patent literature describe high strength and toughness of the half-thickness portion. However, these pieces of non-patent literature do not describe the toughness (Charpy impact characteristics) of the surface of a steel plate. In general, thick-walled materials are manufactured by a quenching and tempering process. The formation of a martensite structure on the surface of a steel plate, on which the cooling rate is higher than in the half-thickness portion, deteriorates the toughness (Charpy impact characteristics) of the surface of the steel plate. However, these pieces of non-patent literature do not describe the manufacture of a steel plate consistently having a tough surface.

The present invention has been made to solve such problems and aims to provide a method for manufacturing a thick-walled high-toughness high-strength steel plate that has high surface toughness and high strength and toughness of the inner part thereof.

### Solution to Problem

In order to solve the problems, the present inventors have extensively studied the microstructure control factors that satisfy high toughness of the surface of a thick-walled steel plate having a yield strength of 620 MPa or more and a thickness of 100 mm or more and also satisfy high strength and toughness of the half-thickness portion of the thick-walled steel plate, and have found the following.
1. When the cooling rate during the solidification of a raw material steel exceeds 1°C/s, microsegregation competes with the solidification reaction. This reduces microsegregation. In the manufacture of a large piece of steel, the cooling rate during the solidification of the steel decreases to 1°C/s or less, and consequently microsegregation becomes noticeable. Even in such a case, in order to achieve high toughness of the surface of a steel plate, on which a martensite structure is formed during quenching, it is important to reduce the P content and microsegregation during solidification. When primary crystals during solidification form a δ phase, and the percentage of the δ phase at the beginning of the formation of a γ phase is 30% or more, this results in reduced microsegregation and improved toughness. The percentage % described above refers to % by volume.
2. In order to achieve high strength and toughness of the half-thickness portion, in which the cooling rate is much lower than on the surface of a steel plate during cooling after hot working, it is important to appropriately select the steel composition (components) so as to form a martensite and/or bainite microstructure even at a low cooling rate. To this end, the alloy components should be appropriately selected, and in particular the carbon equivalent (Ceq) should be 0.65% or more. In addition to the appropriate component design, it is also important to form the desired structure by hot working and heat treatment.
3. Refinement of prior γ grain size is effective in improving toughness. Refinement of prior γ grain size before heat treatment, that is, refinement of prior γ grain size just after hot working is important for refinement of prior γ grain size after heat treatment. Thus, it is important to select appropriate hot working conditions and rolling conditions.

As a result of further investigation of these findings, a method for manufacturing a thick-walled high-toughness high-strength steel plate according to the present invention is defined in claims 1 through 4.

### Advantageous Effects of Invention

The present invention provides a method for manufacturing a thick-walled high-toughness high-strength steel plate having a thickness of 100 mm or more and having a yield strength of 620 MPa or more and high toughness. The thick-walled high-toughness high-strength steel plate can be used to manufacture steel structures having high safety.

### Description of Embodiments

Embodiments of the present invention will be described below. The present invention is not limited to these embodiments.

### <Thick-Walled High-Toughness High-Strength Steel Plate>

A thick-walled high-toughness high-strength steel plate manufactured according to the present invention has a composition containing, on a mass percent basis, C: 0.08% to 0.20%, Si: 0.40% or less (including 0%), Mn: 0.5% to 5.0%, P: 0.010% or less (including 0%), S: 0.0050% or less (including 0%), Cr: 3.0% or less (including 0%), Ni: 0.1% to 5.0%, Al: 0.010% to 0.080%, N: 0.0070% or less (including 0%), and O: 0.0025% or less (including 0%). Each of the components will be described below. The symbol "%" in the component content refers to "% by mass".

### C: 0.08% to 0.20%

C is an element useful for achieving the strength necessary for structural steel at low cost. This effect requires a C content of 0.08% or more. In a steel structure manufactured from a thick-walled high-toughness high-strength steel plate by welding, however, a C content of more than 0.20% significantly deteriorates toughness of the base metal and weld. Thus, the C content has an upper limit of 0.20%. The C content preferably ranges from 0.08% to 0.14%.

### Si: 0.40% or less

Si is added for deoxidation. When another element is added for deoxidation, however, a steel plate according to the present invention does not necessarily contain Si. In a steel structure manufactured from a thick-walled high-toughness high-strength steel plate by welding, a Si content of more than 0.40% significantly deteriorates toughness of the base metal and heat-affected zone. Thus, the Si content is 0.40% or less, preferably 0.05% to 0.3%, more preferably 0.1% to 0.3%.

### Mn: 0.5% to 5.0%

Mn is added to ensure high strength of the base metal. This effect is insufficient at a Mn content of less than 0.5%. A Mn content of more than 5.0% promotes center segregation, results in a larger casting defect of the slab, and deteriorates mechanical properties of the base metal in a steel structure manufactured from a thick-walled high-toughness high-strength steel plate by welding. Thus, the Mn content has an upper limit of 5.0%. The Mn content preferably ranges from 0.6% to 2%, more preferably 0.6% to 1.6%.

### P: 0.010% or less

In a steel structure manufactured from a thick-walled high-toughness high-strength steel plate by welding, a P content of more than 0.010% significantly deteriorates toughness of the base metal and heat-affected zone. Thus, the P content is preferably minimized (may be zero) and is limited to 0.010% or less.

### S: 0.0050% or less

In a steel structure manufactured from a thick-walled high-toughness high-strength steel plate by welding, a S content of more than 0.0050% significantly deteriorates toughness of the base metal and heat-affected zone. Thus, the S content is preferably minimized (may be zero) and is 0.0050% or less.

### Cr: 3.0% or less

Cr is an element effective in strengthening the base metal. However, an excessively high Cr content deteriorates weldability. Thus, the Cr content is 3.0% or less, preferably 0.1% to 2%, more preferably 0.7% to 1.7%. The Cr content may be 0%.

### Ni: 0.1% to 5.0%

Ni is an element useful for improving the strength of steel and the toughness of the heat-affected zone. This effect requires a Ni content of 0.1% or more. However, a Ni content of more than 5.0% significantly deteriorates economic efficiency. Thus, the Ni content has an upper limit of 5.0%. The Ni content preferably ranges from 0.4% to 4%, more preferably 0.8% to 3.8%.

### Al: 0.010% to 0.080%

Al is added for sufficient deoxidation of molten steel. An Al content of less than 0.010% is insufficient for the effect. On the other hand, an Al content of more than 0.080% deteriorates toughness of the base metal due to an increased dissolved Al content in the base metal in a steel structure manufactured from a thick-walled high-toughness high-strength steel plate by welding. Thus, the Al content is 0.080% or less, preferably 0.030% to 0.080%, more preferably 0.030% to 0.070%.

### N: 0.0070% or less

N, together with Ti, forms a nitride and thereby performs refinement of the structure and improves the toughness of the base metal and heat-affected zone in a steel structure manufactured from a thick-walled high-toughness high-strength steel plate by welding. The toughness can be improved by a constituent other than N. Thus, a steel plate according to the present invention does not necessarily contain N. When trying to produce this effect with N, the N content is preferably 0.0015% or more. In a steel structure manufactured from a thick-walled high-toughness high-strength steel plate by welding, however, a N content of more than 0.0070% deteriorates toughness of the base metal due to an increased dissolved N content in the base metal and deteriorates toughness of the heat-affected zone due to the formation of coarse carbonitride. Thus, the N content is 0.0070% or less, preferably 0.006% or less, more preferably 0.005% or less.

### O: 0.0025% or less

An O content of more than 0.0025% significantly deteriorates toughness due to the formation of a hard oxide in steel. Thus, the O content is preferably minimized (may be zero) and is 0.0025% or less.

In addition to these elements, a thick-walled high-toughness high-strength steel plate manufactured according to the present invention can contain at least one of Cu, Mo, V, Nb, and Ti in order to further improve strength and/or toughness.

### Cu: 0.50% or less

Cu can improve the strength of steel without reducing toughness. A Cu content of more than 0.50% may cause a crack on the surface of a steel plate during hot working. Thus, the Cu content, if any, is 0.50% or less.

### Mo: 1.50% or less

Mo contributes to high strength of the base metal in a steel structure manufactured from a thick-walled high-toughness high-strength steel plate by welding. However, a Mo content of more than 1.50% results in increased hardness and deteriorates toughness due to the precipitation of alloy carbide. Thus, the Mo content, if any, has an upper limit of 1.50%. The Mo content preferably ranges from 0.2% to 0.8%.

### V: 0.400% or less

V contributes to improved strength and toughness of the base metal in a steel structure manufactured from a thick-walled high-toughness high-strength steel plate by welding. V precipitates as VN and is effective in decreasing the amount of dissolved N. However, a V content of more than 0.400% deteriorates toughness due to the precipitation of hard VC. Thus, the V content, if any, is preferably 0.400% or less, more preferably 0.01% to 0.1%.

### Nb: 0.100% or less

Nb is effective in improving the strength of the base metal. A Nb content of more than 0.100% deteriorates toughness of the base metal. Thus, the Nb content has an upper limit of 0.100%. The Nb content is preferably 0.025% or less.

### Ti: 0.005% to 0.020%

Ti forms TiN during heating and effectively suppresses the coarsening of austenite. In a steel structure manufactured from a thick-walled high-toughness high-strength steel plate by welding, Ti improves the toughness of the base metal and heat-affected zone. However, a Ti content of more than 0.020% results in coarsening of Ti nitride and deteriorates toughness of the base metal. Thus, the Ti content, if any, ranges from 0.005% to 0.020%, preferably 0.008% to 0.015%.

In addition to these components, a thick-walled high-toughness high-strength steel plate manufactured according to the present invention can further contain at least one of Mg, Ta, Zr, Y, B, Ca, and REM to improve the material quality.

### Mg: 0.0001% to 0.0050%

Mg forms a stable oxide at high temperatures, effectively suppresses the coarsening of prior γ grains in the heat-affected zone, and is effective in improving the toughness of the weld. These effects require a Mg content of 0.0001% or more. However, a Mg content of more than 0.0050% results in an increased number of inclusions and deteriorates toughness. Thus, the Mg content, if any, is preferably 0.0050% or less, more preferably 0.0001% to 0.015%.

### Ta: 0.01% to 0.20%

The addition of an adequate amount of Ta is effective in improving strength. More specifically, a Ta content of 0.01% or more is effective. However, a Ta content of more than 0.20% deteriorates toughness due to formation of precipitates. Thus, the Ta content, if any, ranges from 0.01% to 0.20%.

### Zr: 0.005% to 0.1%

Zr is an element effective in improving strength. A Zr content of 0.005% or more is effective in producing this effect. However, a Zr content of more than 0.1% deteriorates toughness due to the formation of a coarse precipitate. Thus, the Zr content, if any, ranges from 0.005% to 0.1%.

### Y: 0.001% to 0.01%

Y forms a stable oxide at high temperatures, effectively suppresses the coarsening of prior γ grains in the heat-affected zone, and is effective in improving the toughness of the weld. An Y content of 0.001% or more is effective in producing these effects. However, an Y content of more than 0.01% results in an increased number of inclusions and deteriorates toughness. Thus, the Y content, if any, ranges from 0.001% to 0.01%.

### B: 0.0030% or less

B segregates at austenite grain boundaries, suppresses ferrite transformation from the grain boundaries, and improves hardenability. However, a B content of more than 0.0030% deteriorates hardenability and toughness due to the precipitation of B as a carbonitride. Thus, the B content is 0.0030% or less. The B content, if any, preferably ranges from 0.0003% to 0.0030%, more preferably 0.0005% to 0.002%.

### Ca: 0.0005% to 0.0050%

Ca is an element useful for the morphology control of a sulfide inclusion. This effect requires a Ca content of 0.0005% or more. However, a Ca content of more than 0.0050% deteriorates cleanliness and toughness. Thus, the Ca content, if any, is preferably 0.0050% or less, more preferably 0.0005% to 0.0025%.

### REM: 0.0005% to 0.0100%

Like Ca, REM forms an oxide and a sulfide in steel and is effective in improving the material quality. This effect requires a REM content of 0.0005% or more. However, the effect levels off at a REM content of 0.0100% or more. Thus, the REM content, if any, is 0.0100% or less, preferably 0.0005% to 0.005%.

These optional elements in amounts below the lower limits do not reduce the advantages of the present invention. Thus, the optional elements in amounts below the lower limits are considered to be contained as incidental impurities.

### Ceq^{IIW} ≥ 0.65%

In the present invention, an appropriate alloy component needs to be added to ensure that a half-thickness portion of a thick-walled high-toughness high-strength steel plate having a thickness of 100 mm or more has a yield strength of 620 MPa or more and high toughness. More specifically, as represented by the following formula (1), alloying element contents need to be adjusted such that the carbon equivalent (Ceq^{IIW}) is 0.65% or more. ${Ceq}^{IIW} = C + Mn / 6 + \left(Cu+Ni\right) / 15 + \left(Cr+Mo+V\right) / 5 \geq 0.65$

The element symbols in the formula denote the corresponding element contents (% by mass). In the absence of an element, the element symbol is denoted by 0.$\left({C}_{L}-C\right) / {C}_{L} \times 100 \geq 30$

As described later, the present invention provides a steel plate having desirable characteristics even when the steel plate is manufactured from steel casted under conditions where the cooling rate of a slab surface during solidification is 1°C/s or less. In the present invention, microsegregation needs to be reduced to achieve high toughness (vE-40 ≥ 70 J) of the surface of a thick-walled high-toughness high-strength steel plate having a thickness of 100 mm or more, particularly manufactured from steel casted under conditions where the cooling rate of a slab surface during solidification is 1°C/s or less. To this end, primary crystals during solidification need to form a δ phase, and the percentage ((C_{L} - C)/C_{L} x 100) of the δ phase at the beginning of the formation of a γ phase needs to be 30% or more. ${C}_{L} = 0.2 - \left(-0.1\times \left(0.2-Si\right)-0.03\times \left(1.1-Mn\right)-0.12\times \left(0.2-Cu\right)-0.11\times \left(3-Ni\right)+0.025\times \left(1.2-Cr\right)+0.1\times \left(0.5-Mo\right)+0.2\times \left(0.04-V\right)-0.05\times \left(0.06-Al\right)\right)$

In the formula (3), the element symbols denote the respective alloy component contents (% by mass), and in the absence of an element, the element symbol is denoted by 0.

In order to form a δ phase, the C content needs to be specified depending on each component other than C, such as Si or Mn. The effects of an alloying element on the C solid solubility limit (C_{L}) of the δ phase were calculated using thermodynamic calculation software "Thermo-Calc". The result was used to determine the factor. For example, the factor "-0.1" for "Si" means that 1% Si decreases the C solid solubility limit of the δ phase by 0.1%, and the C content of the base metal needs to be decreased to achieve the required percentage of the δ phase. In the present invention, the calculation of C_{L} was based on the component of C: 0.12%, Si: 0.2%, Mn: 1.1%, Cu: 0.2%, Cr: 1.2%, Ni: 3%, Mo: 0.5%, V: 0.04% and Al: 0.06%, and the factors for the calculation of C_{L} were determined by calculating a variation from the dissolved C content caused by a variation in each alloying element content. When the percentage (C_{L} - C)/C_{L} x 100 of C to be added relative to the C solid solubility limit in the δ phase thus calculated is 30% or more, the percentage of the δ phase at the beginning of the formation of the γ phase can be 30% or more.

In the present invention, in order to ensure the safety of steel during use, the reduction of area in the thickness direction at half the thickness of the plate is 40% or more when measured by a method described in the example.

### <Method for Manufacturing Thick-Walled High-Toughness High-Strength Steel Plate>

The manufacturing conditions in the present invention will be described below. In the description, the temperature "°C" refers to the temperature in the half-thickness portion except for the quenching temperature in the case of quenching without leaving to cool after rolling. The quenching temperature in the case of quenching without leaving to cool after rolling is the surface temperature of the steel plate. This is because the temperature distribution of the steel plate in the thickness direction increases during rolling, and a decrease in the surface temperature of the steel plate needs to be considered. The temperature of the half-thickness portion is determined, for example, by simulation calculation from the thickness, surface temperature, and cooling conditions. For example, the temperature of the half-thickness portion is determined by calculating the temperature distribution in the thickness direction using finite difference methods.

### Steel

A molten steel having the composition described above is produced by a conventional method, such as with a converter, an electric furnace, or a vacuum melting furnace, and is formed into a piece of steel, such as a slab or billet, by a conventional casting method, such as a continuous casting process or an ingot casting process. The cooling rate during solidification is determined by direct measurement with a thermocouple or by simulation calculation, such as heat-transfer calculation. As described above, in the present invention, steel manufactured under conditions where the cooling rate of a surface during solidification is 1°C/s or less can preferably be used.

When the loads of a forging machine and a rolling mill and so on are restricted, the thickness of the material may be reduced by slabbing.

### Hot-Forging Conditions for Steel

A cast bloom or steel bloom having the composition described above is heated to a temperature in the range of 1200°C to 1350°C. A reheating temperature of less than 1200°C results in not only an insufficient rolling reduction due to an increased load to achieve a predetermined cumulative rolling reduction in hot working but also low production efficiency due to additional heating as required during working. Thus, the reheating temperature is 1200°C or more. A large amount of additive alloying element as steel having a carbon equivalent of 0.65% or more according to the present invention results in a casting defect such as a center porosity or porous shrinkage cavity, having a much increased size in steel. In order to make them harmless by pressure bonding, the cumulative rolling reduction needs to be 25% or more. On the other hand, a reheating temperature of more than 1350°C results in excessive energy consumption, increased likelihood of occurrence of surface flaws due to scales during heating, and increased repair load after hot forging. Thus, the upper limit is 1350°C.

### Slabbing Conditions for Steel

A cast bloom or steel bloom having the composition described above is heated to a temperature in the range of 1200°C to 1350°C. A reheating temperature of less than 1200°C results in not only an insufficient rolling reduction due to an increased load to achieve a predetermined cumulative rolling reduction in hot working but also low production efficiency due to additional heating as required during working. Thus, the reheating temperature is 1200°C or more. In order to make casting defects harmless by pressure bonding and to provide the advantages of the present invention, the cumulative rolling reduction is 30% or more, preferably 40% or more in terms of good reduction of area (RA). On the other hand, a reheating temperature of more than 1350°C results in excessive energy consumption, increased likelihood of surface flaws due to scales during heating, and increased repair load after hot forging. Thus, the upper limit is 1350°C.

### Reheating of Steel after Forging or after Slabbing

Steel after forging is heated to an Ac3 transformation temperature or more and 1200°C or less in order that the steel may have a uniform austenite structure alone. The heating temperature preferably ranges from 1000°C to 1200°C.

The Ac3 transformation temperature is calculated using the following formula (4). $Ac 3 = 937.2 - 476.5 C + 56 Si - 19.7 Mn - 16.3 Cu - 26.6 Ni - 4.9 Cr + 38.1 Mo + 124.8 V + 136.3 Ti + 198.4 Al + 3315 B$

The element symbols in the formula (4) denote the respective alloy component contents (% by mass).

### Hot Rolling Conditions

Steel is hot-rolled to form a plate having a desired thickness. In order to ensure desirable mechanical properties of a half-thickness portion of a thick-walled steel plate having a thickness of 100 mm or more, it is necessary to adjust the steel in the rolling step in order to sufficiently elicit an effect of adjusting and refining of the prior γ grain size. More specifically, rolling at a cumulative rolling reduction of 40% or more can adjust the grain size in the rolling step even in the half-thickness portion in which recrystallization rarely occurs in processing.

### Heat-Treatment Conditions

In order to achieve high strength and toughness of a half-thickness portion, in the present invention, a steel plate is left to cool (for example, air cooling) after hot rolling or is rapidly cooled from the Ar3 temperature or more to 350°C or less without leaving to cool after hot rolling. When the steel plate is left to cool, the steel plate is reheated to the Ac3 temperature to 1050°C and is rapidly cooled from the Ac3 temperature or more to 350°C or less. The reason for the reheating temperature of 1050°C or less is that reheating at a high temperature of more than 1050°C results in coarsening of austenite grains and significantly deteriorates toughness of the base metal in a steel structure manufactured from a thick-walled high-toughness high-strength steel plate by welding. The reheating temperature is the Ac3 temperature or more in order that the steel plate may entirely have an austenite structure. The quenching temperature is the Ac3 temperature or more because the desirable characteristics are not obtained at a temperature below the Ac3 temperature due to the formation of a nonuniform structure composed of ferrite and austenite. In the case of rapid cooling without leaving to cool, the quenching temperature is the Ar3 temperature or more for quenching from the austenite single phase region. The rapid cooling stop temperature is a lower temperature selected from 350°C or less and the Ar3 temperature or less in order to ensure that the steel plate entirely has a transformed structure. The stop temperature should be the Ar3 temperature or less and 350°C or less.

The Ar3 transformation temperature is calculated using the following formula (5). $Ar 3 = 910 - 310 C - 80 Mn - 20 Cu - 15 Cr - 55 Ni - 80 Mo$

The element symbols in the formula (5) denote the respective alloy component contents (% by mass).

In general, the rapid cooling method is industrially water cooling. It is desirable that the cooling rate be as high as possible. Thus, the cooling method is not necessarily water cooling and may be gas cooling, for example.

### Tempering Conditions

The reason for tempering at a temperature in the range of 450°C to 700°C after rapid cooling is described below. Residual stress is not effectively relieved at less than 450°C. On the other hand, a temperature of more than 700°C results in precipitation of various carbides and coarsens the structure of the base metal and deteriorates strength and toughness of the base metal in a steel structure manufactured from a thick-walled high-toughness high-strength steel plate by welding.

Industrially, quenching is sometimes repeated to strengthen steel. Although quenching may be repeated also in the present invention, final quenching requires rapid cooling to 350°C or less after heating to the Ac3 temperature to 1050°C and requires subsequent tempering at 450°C to 700°C.

### EXAMPLES

Steel plate samples No. 1 to No. 38 were manufactured by melting and casting steel No. 1 to No. 30 listed in Table 1 under the conditions listed in Table 2, performing hot forging (except for the samples No. 5, No. 6, and No. 41) or slabbing (the samples No. 5, No. 6, and No. 41), hot-rolling the steel to form a steel plate having a thickness listed in Table 2, and subjecting the steel plate to water quenching and tempering. The steel plate samples No. 1 to No. 38 were subjected to the following tests. In reheating and quenching in this example, the reheating temperature corresponds to the quenching temperature.

The percentage of the δ phase is calculated using the formula (2) from C_{L} calculated using the formula (3) with each base metal component and the C content of the base metal.

The cooling rate during solidification in the manufacture of steel is determined by heat-transfer calculation from the mold surface temperature data measured with a radiation thermometer.

### Tensile Test

A round bar tensile test piece (φ12.5 mm, GL 50 mm) was taken from the half-thickness portion of each steel plate in the direction perpendicular to the rolling direction and was measured in terms of yield strength (YS) and tensile strength (TS).

### Charpy Impact Test

Three 2-mm V-notched Charpy impact test specimens were taken from each surface and half-thickness portion of the steel plates. The rolling direction was the longitudinal direction. The absorbed energies of the test specimens were measured at a test temperature of -40°C in a Charpy impact test and were averaged (the average value for the test specimens taken from the half-thickness portion and the average value for the test specimens taken from the surface).

### Tensile Test in Thickness Direction

A round bar tensile test piece (φ10 mm) was taken from a region including the half-thickness portion of each steel plate in the thickness direction and was measured in terms of reduction of area (RA). The reduction of area is the percentage of the difference between the minimum cross-sectional area after the test specimen was broken and the original cross-sectional area relative to the original cross-sectional area.

Table 2 shows the test results. The results showed that the steel plates of the examples having a steel composition according to the present invention (samples No. 1 to No. 21 and No. 41) had YS of 620 MPa or more, TS of 720 MPa or more, and toughness (vE-40) of 70 J or more at -40°C in the surface and half-thickness portion of the base metal, showing high strength and toughness of the base metal. A comparison between Nos. 5 and 6 and No. 41 showed that reduction of area (RA) was also satisfactory under particular slabbing conditions.

In contrast, in the steel plates according to comparative examples having a composition outside the scope of the present invention (samples No. 22 to No. 32), the base metal had at least one of YS of less than 620 MPa, TS of less than 720 MPa, and toughness (vE-40) of less than 70 J, thus deteriorating characteristics.

As in samples No. 33 to No. 40, even if steel plates had a steel composition according to the present invention, steel plates manufactured under the conditions outside the scope of the present invention had at least one deterioration in YS, TS, and toughness (vE-40) .

**[Table 2]**

| Category | Sample No. | Steel ingot No. | Thickness of material (mm) | Cooling rate during solidification °C/s | Hot forging or slabbing | | Hot rolling | | Thickness of product (mm) | Type of heat treatment | Final heat treatment conditions | | | Mechanical properties of base metal (1/2t) | | | | Toughness of base metal (surface) |
|---|---|---|---|---|---|---|---|---|---|---|---|---|---|---|---|---|---|---|
| | | | | | Heating (°C) | Cumulative rolling reduction (%) | Heating (°C) | Cumulative rolling reduction (%) | | | Quenching temperature (°C) | Cooling stop (°C) | Tempering (°C) | YS (MPa) | TS (MPa) | vE-40 (J) | Tensile RA in thickness direction RA (%) | vE-40 (J) |
| | 1 | 1 | 1000 | 0.32 | 1270 | 80 | 1130 | 43 | 100 | Direct quenching | 850 | 150 | 630 | 695 | 786 | 108 | 73 | 98 |
| | 2 | 2 | 500 | 0.64 | 1230 | 65 | 1130 | 43 | 100 | Reheating quenching | 930 | 100 | 650 | 698 | 795 | 167 | 63 | 105 |
| | 3 | 3 | 300 | 0.90 | 1200 | 30 | 1130 | 50 | 100 | Reheating quenching | 930 | 100 | 630 | 725 | 793 | 102 | 70 | 116 |
| | 4 | 4 | 1000 | 0.33 | 1270 | 70 | 1160 | 43 | 150 | Reheating quenching | 900 | 100 | 630 | 785 | 856 | 205 | 65 | 221 |
| | 5 | 4 | 1000 | 0.33 | 1320 | 55 | 1200 | 53 | 210 | Reheating quenching | 900 | 100 | 630 | 743 | 829 | 145 | 71 | 124 |
| | 6 | 4 | 1000 | 0.33 | 1300 | 55 | 1180 | 67 | 150 | Direct quenching | 860 | 100 | 630 | 751 | 832 | 126 | 58 | 159 |
| | 7 | 5 | 500 | 0.61 | 1270 | 45 | 1160 | 43 | 150 | Reheating quenching | 900 | 100 | 630 | 725 | 821 | 153 | 63 | 205 |
| | 8 | 6 | 1000 | 0.32 | 1270 | 55 | 1130 | 60 | 180 | Reheating quenching | 880 | 100 | 630 | 705 | 816 | 238 | 61 | 211 |
| | 9 | 7 | 1000 | 0.31 | 1270 | 55 | 1130 | 53 | 210 | Reheating quenching | 880 | 100 | 650 | 756 | 864 | 216 | 63 | 163 |
| | 10 | 8 | 1000 | 0.31 | 1300 | 55 | 1130 | 53 | 210 | Reheating quenching | 880 | 100 | 650 | 741 | 836 | 193 | 60 | 121 |
| Example | 11 | 9 | 1000 | 0.30 | 1270 | 55 | 1130 | 53 | 210 | Reheating quenching | 880 | 100 | 650 | 759 | 857 | 186 | 62 | 101 |
| | 12 | 10 | 1200 | 0.25 | 1270 | 55 | 1160 | 50 | 250 | Reheating quenching | 900 | 100 | 630 | 748 | 852 | 221 | 59 | 146 |
| | 13 | 11 | 1000 | 0.29 | 1270 | 70 | 1160 | 43 | 150 | Reheating quenching | 880 | 100 | 630 | 728 | 839 | 169 | 71 | 101 |
| | 14 | 12 | 1300 | 0.19 | 1270 | 60 | 1160 | 50 | 250 | Reheating quenching | 880 | 100 | 660 | 793 | 912 | 221 | 68 | 145 |
| | 15 | 13 | 1200 | 0.32 | 1270 | 85 | 1130 | 43 | 100 | Reheating quenching | 930 | 100 | 650 | 665 | 756 | 103 | 73 | 126 |
| | 16 | 14 | 1000 | 0.31 | 1270 | 55 | 1160 | 53 | 210 | Reheating quenching | 880 | 100 | 650 | 723 | 814 | 203 | 69 | 163 |
| | 17 | 15 | 1000 | 0.32 | 1270 | 55 | 1160 | 53 | 210 | Reheating quenching | 1050 | 150 | 670 | 641 | 738 | 145 | 70 | 101 |
| | 18 | 16 | 500 | 0.64 | 1230 | 65 | 1130 | 43 | 100 | Reheating quenching | 930 | 100 | 650 | 732 | 841 | 167 | 77 | 83 |
| | 19 | 17 | 500 | 0.65 | 1230 | 65 | 1160 | 43 | 100 | Reheating quenching | 900 | 100 | 650 | 703 | 789 | 196 | 73 | 113 |
| | 20 | 18 | 300 | 0.91 | 1200 | 40 | 1160 | 43 | 100 | Direct quenching | 880 | 150 | 650 | 752 | 846 | 138 | 65 | 106 |
| | 21 | 19 | 1000 | 0.29 | 1350 | 50 | 1160 | 50 | 250 | Reheating quenching | 900 | 100 | 650 | 746 | 863 | 231 | 62 | 93 |
| | 22 | 20 | 1000 | 0.29 | 1270 | 55 | 1160 | 53 | 210 | Reheating quenching | 880 | 100 | 640 | 716 | 815 | 196 | 61 | 43 |
| | 23 | 21 | 300 | 0.92 | 1200 | 40 | 1160 | 43 | 100 | Reheating quenching | 930 | 100 | 650 | 589 | 695 | 22 | 69 | 121 |
| | 24 | 22 | 1000 | 0.31 | 1270 | 70 | 1160 | 43 | 150 | Reheating quenching | 900 | 100 | 630 | 845 | 956 | 19 | 62 | 96 |
| | 25 | 23 | 1000 | 0.29 | 1270 | 70 | 1160 | 43 | 150 | Reheating quenching | 930 | 100 | 630 | 547 | 663 | 21 | 68 | 124 |
| | 26 | 24 | 1000 | 0.29 | 1270 | 55 | 1130 | 53 | 210 | Reheating quenching | 930 | 100 | 650 | 728 | 823 | 41 | 64 | 39 |
| | 27 | 25 | 1200 | 0.24 | 1270 | 55 | 1160 | 50 | 250 | Reheating quenchinq | 880 | 100 | 630 | 802 | 915 | 23 | 51 | 96 |
| | 28 | 26 | 1000 | 0.28 | 1270 | 70 | 1160 | 43 | 150 | Reheating quenching | 880 | 100 | 630 | 731 | 829 | 32 | 57 | 23 |
| | 29 | 27 | 1000 | 0.31 | 1270 | 55 | 1130 | 53 | 210 | Reheating quenching | 900 | 100 | 650 | 741 | 854 | 35 | 63 | 31 |
| | 30 | 28 | 000 | 0.29 | 1270 | 55 | 1130 | 53 | 210 | Reheating quenching | 900 | 100 | 650 | 796 | 921 | 43 | 61 | 89 |
| Comparative example | 31 | 29 | 1000 | 0.32 | 1270 | 55 | 1130 | 53 | 210 | Reheating quenching | 900 | 100 | 650 | 732 | 816 | 48 | 72 | 56 |
| | 32 | 30 | 1000 | 0.31 | 1270 | 70 | 1160 | 43 | 150 | Reheating quenching | 900 | 100 | 630 | 698 | 784 | 61 | 70 | 52 |
| | 33 | 3 | 300 | 0.91 | 1200 | 15 | 1130 | 60 | 100 | Reheating quenching | 930 | 100 | 630 | 716 | 804 | 43 | 23 | 115 |
| | 34 | 3 | 300 | 0.89 | 1200 | 55 | 1130 | 20 | 100 | Reheating quenching | 930 | 100 | 630 | 722 | 816 | 45 | 35 | 96 |
| | 35 | 3 | 300 | 0.90 | 1200 | 30 | 1130 | 50 | 100 | Reheating quenching | 1100 | 100 | 630 | 735 | 824 | 36 | 53 | 49 |
| | 36 | 3 | 300 | 0.92 | 1200 | 30 | 1130 | 50 | 100 | Reheating quenching | 840 | 100 | 630 | 536 | 646 | 46 | 49 | 52 |
| | 37 | 3 | 300 | 0.90 | 1200 | 30 | 1130 | 50 | 100 | Direct quenchinq | 623 | 100 | 630 | 596 | 683 | 52 | 51 | 61 |
| | 38 | 3 | 300 | 0.91 | 1200 | 30 | 130 | 50 | 100 | Reheating quenching | 930 | 400 | 630 | 503 | 641 | 32 | 64 | 103 |
| | 39 | 3 | 300 | 0.90 | 1200 | 30 | 1130 | 50 | 100 | Reheating quenching | 930 | 100 | 720 | 569 | 657 | 153 | 68 | 146 |
| | 40 | 3 | 300 | 0.91 | 1200 | 30 | 1130 | 50 | 100 | Reheating quenching | 930 | 100 | 400 | 793 | 902 | 41 | 63 | 53 |
| Comparative Example | 41 | 5 | 500 | 0.61 | 1300 | 30 | 1180 | 40 | 210 | Reheating quenching | 900 | 100 | 600 | 683 | 766 | 105 | 29 | 192 |

## Claims

1. A method for manufacturing a thick-walled high-toughness high-strength steel plate having a thickness of 100 mm or more, a yield strength of 620 MPa or more, and comprising, on a mass percent basis,
C: 0.08% to 0.20%,
Si: 0.40% or less,
Mn: 0.5% to 5.0%,
P: 0.010% or less,
S: 0.0050% or less,
Cr: 3.0% or less,
Ni: 0.1% to 5.0%,
Al: 0.010% to 0.080%,
N: 0.0070% or less, and
O: 0.0025% or less,
following formulae (1) and (2) being satisfied, optionally at least one of
Cu: 0.50% or less,
Mo: 1.50% or less,
V: 0.400% or less,
Nb: 0.100% or less,
Ti: 0.005% to 0.020%,
Mg: 0.0001% to 0.0050%,
Ta: 0.01% to 0.20%,
Zr: 0.005% to 0.1%,
Y: 0.001% to 0.01%,
B: 0.0030% or less,
Ca: 0.0005% to 0.0050%, and
REM: 0.0005% to 0.0100%,
a remainder being Fe and incidental impurities, and comprising a toughness (vE-40) of 70 J or more at -40°C in the surface portion of the base metal: ${Ceq}^{IIW} = C + Mn / 6 + \left(Cu+Ni\right) / 15 + \left(Cr+Mo+V\right) / 5 \geq 0.65$ $\left({C}_{L}-C\right) / {C}_{L} \times 100 \geq 30$ wherein C_{L} is defined by the following formula: ${C}_{L} = 0.2 - \left(-0.1\times \left(0.2-Si\right)-0.03\times \left(1.1-Mn\right)-0.12\times \left(0.2-Cu\right)-0.11\times \left(3-Ni\right)+0.025\times \left(1.2-Cr\right)+0.1\times \left(0.5-Mo\right)+0.2\times \left(0.04-V\right)-0.05\times \left(0.06-Al\right)\right)$ wherein element symbols in the formulae denote the respective alloy component contents (% by mass), and in the absence of an element the element symbol is denoted by 0, and wherein
a reduction of area in a thickness direction at half the thickness of the plate, which is the percentage of the difference between the minimum cross-sectional area after a round bar tensile test specimen including the half-thickness portion of the steel plate in the thickness direction is broken in a tensile test and the original cross-sectional area relative to the original cross-sectional area, is 40% or more,
wherein the method comprises:
heating steel to 1200°C to 1350°C,
hot-forging the steel at a cumulative reduction of 25% or more,
heating the steel to an Ac3 temperature or more and 1200°C or less,
hot-rolling the steel at a cumulative rolling reduction of 40% or more,
leaving the steel to cool,
reheating the steel to the Ac3 temperature or more and 1050°C or less,
rapidly cooling the steel from the Ac3 temperature or more to a lower temperature, which is both 350°C or less and an Ar3 temperature or less, and
tempering the steel at a temperature in the range of 450°C to 700°C.

2. A method for manufacturing a thick-walled high-toughness high-strength steel plate having a thickness of 100 mm or more, a yield strength of 620 MPa or more, and comprising, on a mass percent basis,
C: 0.08% to 0.20%,
Si: 0.40% or less,
Mn: 0.5% to 5.0%,
P: 0.010% or less,
S: 0.0050% or less,
Cr: 3.0% or less,
Ni: 0.1% to 5.0%,
Al: 0.010% to 0.080%,
N: 0.0070% or less, and
O: 0.0025% or less,
following formulae (1) and (2) being satisfied, optionally at least one of
Cu: 0.50% or less,
Mo: 1.50% or less,
V: 0.400% or less,
Nb: 0.100% or less,
Ti: 0.005% to 0.020%,
Mg: 0.0001% to 0.0050%,
Ta: 0.01% to 0.20%,
Zr: 0.005% to 0.1%,
Y: 0.001% to 0.01%,
B: 0.0030% or less,
Ca: 0.0005% to 0.0050%, and
REM: 0.0005% to 0.0100%,
a remainder being Fe and incidental impurities, and comprising a toughness (vE-40) of 70 J or more at -40°C in the surface portion of the base metal: ${Ceq}^{IIW} = C + Mn / 6 + \left(Cu+Ni\right) / 15 + \left(Cr+Mo+V\right) / 5 \geq 0.65$ $\left({C}_{L}-C\right) / {C}_{L} \times 100 \geq 30$ wherein C_{L} is defined by the following formula: ${C}_{L} = 0.2 - \left(-0.1\times \left(0.2-Si\right)-0.03\times \left(1.1-Mn\right)-0.12\times \left(0.2-Cu\right)-0.11\times \left(3-Ni\right)+0.025\times \left(1.2-Cr\right)+0.1\times \left(0.5-Mo\right)+0.2\times \left(0.04-V\right)-0.05\times \left(0.06-Al\right)\right)$ wherein element symbols in the formulae denote the respective alloy component contents (% by mass), and in the absence of an element the element symbol is denoted by 0, and wherein
a reduction of area in a thickness direction at half the thickness of the plate, which is the percentage of the difference between the minimum cross-sectional area after a round bar tensile test specimen including the half-thickness portion of the steel plate in the thickness direction is broken in a tensile test and the original cross-sectional area relative to the original cross-sectional area, is 40% or more,
wherein the method comprises:
heating steel to 1200°C to 1350°C,
hot-forging the steel at a cumulative reduction of 25% or more,
heating the steel to an Ac3 temperature or more and 1200°C or less,
hot-rolling the steel at a cumulative rolling reduction of 40% or more,
rapidly cooling the steel from an Ar3 temperature or more to a lower temperature which is both 350°C or less and the Ar3 temperature or less, and
tempering the steel at a temperature in the range of 450°C to 700°C.

3. A method for manufacturing a thick-walled high-toughness high-strength steel plate having a thickness of 100 mm or more, a yield strength of 620 MPa or more, and comprising, on a mass percent basis,
C: 0.08% to 0.20%,
Si: 0.40% or less,
Mn: 0.5% to 5.0%,
P: 0.010% or less,
S: 0.0050% or less,
Cr: 3.0% or less,
Ni: 0.1% to 5.0%,
Al: 0.010% to 0.080%,
N: 0.0070% or less, and
O: 0.0025% or less,
following formulae (1) and (2) being satisfied, optionally at least one of
Cu: 0.50% or less,
Mo: 1.50% or less,
V: 0.400% or less,
Nb: 0.100% or less,
Ti: 0.005% to 0.020%,
Mg: 0.0001% to 0.0050%,
Ta: 0.01% to 0.20%,
Zr: 0.005% to 0.1%,
Y: 0.001% to 0.01%,
B: 0.0030% or less,
Ca: 0.0005% to 0.0050%, and
REM: 0.0005% to 0.0100%,
a remainder being Fe and incidental impurities, and comprising a toughness (vE-40) of 70 J or more at -40°C in the surface portion of the base metal: ${Ceq}^{IIW} = C + Mn / 6 + \left(Cu+Ni\right) / 15 + \left(Cr+Mo+V\right) / 5 \geq 0.65$ $\left({C}_{L}-C\right) / {C}_{L} \times 100 \geq 30$ wherein C_{L} is defined by the following formula: ${C}_{L} = 0.2 - \left(-0.1\times \left(0.2-Si\right)-0.03\times \left(1.1-Mn\right)-0.12\times \left(0.2-Cu\right)-0.11\times \left(3-Ni\right)+0.025\times \left(1.2-Cr\right)+0.1\times \left(0.5-Mo\right)+0.2\times \left(0.04-V\right)-0.05\times \left(0.06-Al\right)\right)$ wherein element symbols in the formulae denote the respective alloy component contents (% by mass), and in the absence of an element the element symbol is denoted by 0, and wherein
a reduction of area in a thickness direction at half the thickness of the plate, which is the percentage of the difference between the minimum cross-sectional area after a round bar tensile test specimen including the half-thickness portion of the steel plate in the thickness direction is broken in a tensile test and the original cross-sectional area relative to the original cross-sectional area, is 40% or more,
wherein the method comprises:
heating steel to 1200°C to 1350°C,
slabbing the steel at a cumulative rolling reduction of 40% or more,
heating the steel to an Ac3 temperature or more and 1200°C or less,
hot-rolling the steel at a cumulative rolling reduction of 40% or more, leaving the steel to cool,
reheating the steel to the Ac3 temperature or more and 1050°C or less,
rapidly cooling the steel from the Ac3 temperature or more to a lower temperature which is both 350°C or less and an Ar3 temperature or less, and
tempering the steel at a temperature in the range of 450°C to 700°C.

4. A method for manufacturing a thick-walled high-toughness high-strength steel plate having a thickness of 100 mm or more, a yield strength of 620 MPa or more, and comprising, on a mass percent basis,
C: 0.08% to 0.20%,
Si: 0.40% or less,
Mn: 0.5% to 5.0%,
P: 0.010% or less,
S: 0.0050% or less,
Cr: 3.0% or less,
Ni: 0.1% to 5.0%,
Al: 0.010% to 0.080%,
N: 0.0070% or less, and
O: 0.0025% or less,
following formulae (1) and (2) being satisfied, optionally at least one of
Cu: 0.50% or less,
Mo: 1.50% or less,
V: 0.400% or less,
Nb: 0.100% or less,
Ti: 0.005% to 0.020%,
Mg: 0.0001% to 0.0050%,
Ta: 0.01% to 0.20%,
Zr: 0.005% to 0.1%,
Y: 0.001% to 0.01%,
B: 0.0030% or less,
Ca: 0.0005% to 0.0050%, and
REM: 0.0005% to 0.0100%,
a remainder being Fe and incidental impurities, and comprising a toughness (vE-40) of 70 J or more at -40°C in the surface portion of the base metal: ${Ceq}^{IIW} = C + Mn / 6 + \left(Cu+Ni\right) / 15 + \left(Cr+Mo+V\right) / 5 \geq 0.65$ $\left({C}_{L}-C\right) / {C}_{L} \times 100 \geq 30$ wherein C_{L} is defined by the following formula: ${C}_{L} = 0.2 - \left(-0.1\times \left(0.2-Si\right)-0.03\times \left(1.1-Mn\right)-0.12\times \left(0.2-Cu\right)-0.11\times \left(3-Ni\right)+0.025\times \left(1.2-Cr\right)+0.1\times \left(0.5-Mo\right)+0.2\times \left(0.04-V\right)-0.05\times \left(0.06-Al\right)\right)$ wherein element symbols in the formulae denote the respective alloy component contents (% by mass), and in the absence of an element the element symbol is denoted by 0, and wherein
a reduction of area in a thickness direction at half the thickness of the plate, which is the percentage of the difference between the minimum cross-sectional area after a round bar tensile test specimen including the half-thickness portion of the steel plate in the thickness direction is broken in a tensile test and the original cross-sectional area relative to the original cross-sectional area, is 40% or more,
wherein the method comprises:
heating steel to 1200°C to 1350°C,
slabbing the steel at a cumulative rolling reduction of 40% or more,
heating the steel to an Ac3 temperature or more and 1200°C or less,
hot-rolling the steel at a cumulative rolling reduction of 40% or more,
rapidly cooling the steel from an Ar3 temperature or more to a lower temperature, which is both 350°C or less and the Ar3 temperature or less, and
tempering the steel at a temperature in the range of 450°C to 700°C.

## Patentansprüche

1. Verfahren zum Herstellen eines dickwandigen, hochzähen, hochfesten Stahlblechs mit einer Dicke von 100 mm oder mehr, einer Dehngrenze von 620 MPa oder mehr, das in Masse-% umfasst:
0,08% bis 0,20% C,
0,40% oder weniger Si,
0,5% bis 5,0% Mn,
0,010 % oder weniger P,
0,0050% oder weniger S,
3,0% oder weniger Cr,
0,1% bis 5,0% Ni,
0,010% bis 0,080% Al,
0,0070% oder weniger N, sowie
0,0025% oder weniger O,
wenn die Formeln (1) und (2) gelten, optional
0,50 % oder weniger Cu,
1,50% oder weniger Mo,
0,400% oder weniger V,
0,100% oder weniger Nb,
0,005% bis 0,020% Ti,
0,0001% bis 0,0050% Mg,
0,01% bis 0,20% Ta,
0,005% bis 0,1% Zr,
0,001% bis 0,01% Y,
0,0030% oder weniger B,
0,0005% bis 0,0050% Ca, oder/und
0,0005% bis 0,0100% REM,
wobei ein Rest Fe und zufällige Verunreinigungen sind, und es eine Zähigkeit (vE-40) von 70 J oder mehr bei -40 °C in dem Oberflächenabschnitt des Grundmetalls aufweist: ${Ceq}^{IIW} = C + Mn / 6 + \left(Cu+Ni\right) / 15 + \left(Cr+Mo+V\right) / 5 \geq 0,65$ $\left({C}_{L}-C\right) / {C}_{L} \times 100 \geq 30$ wobei C_{L} durch die folgende Formel definiert wird: ${C}_{L} = 0,2 - \left(-0,1\times \left(0,2-Si\right)-0,03\times \left(1,1-Mn\right)-0,12\times \left(0,2-Cu\right)-0,11\times \left(3-Ni\right)+0,025\times \left(1,2-Cr\right)+0,1\times \left(0,5-Mo\right)+0,2\times \left(0,04-V\right)-0,05\times \left(0,06-Al\right)\right)$ wobei Element-Symbole in den Formeln den Gehalt (Masse-%) des jeweiligen Legierungsbestandteils angeben, und beim Nichtvorhandensein eines Elementes das Element-Symbol mit 0 angegeben wird, und
eine Querschnittsverminderung in einer Dickenrichtung bei der halben Blechdicke, die der prozentuale Anteil der Differenz zwischen der minimalen Querschnittsfläche, nachdem ein Zugversuch-Prüfkörper in Form eines Rundstabes, der den Abschnitt mit halber Dicke des Stahlblechs in der Dickenrichtung einschließt, in einem Zugversuch gebrochen war, und der ursprünglichen Querschnittsfläche relativ zu der ursprünglichen Querschnittsfläche ist, 40 % oder mehr beträgt,
wobei das Verfahren umfasst:
Erhitzen von Stahl auf 1200 °C bis 1350 °C,
Warmschmieden des Stahls mit einer kumulativen Reduktion von 25% oder mehr,
Erhitzen des Stahls auf eine Ac3-Temperatur oder darüber und 1200 °C oder darunter,
Warmwalzen des Stahls mit einer kumulativen Walzreduktion von 40% oder mehr,
Abkühlen des Stahls,
erneutes Erhitzen des Stahls auf die Ac3-Temperatur oder darüber und 1050 °C oder darunter,
schnelles Abkühlen des Stahls von der Ac3-Temperatur oder darüber auf eine niedrigere Temperatur, die sowohl auf 350 °C oder darunter als auch auf einer Ar3-Temperatur oder darunter liegt, und
Anlassen des Stahls bei einer Temperatur im Bereich von 450 °C bis 700 °C.

2. Verfahren zum Herstellen eines dickwandigen, hochzähen, hochfesten Stahlblechs mit einer Dicke von 100 mm oder mehr, einer Dehngrenze von 620 MPa oder mehr, das in Masse-% umfasst:
0,08% bis 0,20% C,
0,40% oder weniger Si,
0,5% bis 5,0% Mn,
0,010 % oder weniger P,
0,0050% oder weniger S,
3,0% oder weniger Cr,
0,1% bis 5,0% Ni,
0,010% bis 0,080% Al,
0,0070% oder weniger N, sowie
0,0025% oder weniger O,
wenn die Formeln (1) und (2) gelten, optional
0,50 % oder weniger Cu,
1,50% oder weniger Mo,
0,400% oder weniger V,
0,100% oder weniger Nb,
0,005% bis 0,020% Ti,
0,0001% bis 0,0050% Mg,
0,01% bis 0,20% Ta,
0,005% bis 0,1% Zr,
0,001% bis 0,01% Y,
0,0030% oder weniger B,
0,0005% bis 0,0050% Ca, oder/und
0,0005% bis 0,0100% REM,
wobei ein Rest Fe und zufällige Verunreinigungen sind, und es eine Zähigkeit (vE-40) von 70 J oder mehr bei -40 °C in dem Oberflächenabschnitt des Grundmetalls aufweist: ${Ceq}^{IIW} = C + Mn / 6 + \left(Cu+Ni\right) / 15 + \left(Cr+Mo+V\right) / 5 \geq 0,65$ $\left({C}_{L}-C\right) / {C}_{L} \times 100 \geq 30$ wobei C_{L} durch die folgende Formel definiert wird: ${C}_{L} = 0,2 - \left(-0,1\times \left(0,2-Si\right)-0,03\times \left(1,1-Mn\right)-0,12\times \left(0,2-Cu\right)-0,11\times \left(3-Ni\right)+0,025\times \left(1,2-Cr\right)+0,1\times \left(0,5-Mo\right)+0,2\times \left(0,04-V\right)-0,05\times \left(0,06-Al\right)\right)$ wobei Element-Symbole in den Formeln den Gehalt (Masse-%) der jeweiligen Legierungsbestandteile angeben, und beim Nichtvorhandensein eines Elementes das Element-Symbol mit 0 angegeben wird, und
eine Querschnittsverminderung in einer Dickenrichtung bei der halben Blechdicke, die der prozentuale Anteil der Differenz zwischen der minimalen Querschnittsfläche, nachdem ein Zugversuch-Prüfkörper in Form eines Rundstabes, der den Abschnitt mit halber Dicke des Stahlblechs in der Dickenrichtung einschließt, in einem Zugversuch gebrochen war, und der ursprünglichen Querschnittsfläche relativ zu der ursprünglichen Querschnittsfläche ist, 40 % oder mehr beträgt,
wobei das Verfahren umfasst:
Erhitzen von Stahl auf 1200 °C bis 1350 °C,
Warmschmieden des Stahls mit einer kumulativen Reduktion von 25% oder mehr,
Erhitzen des Stahls auf eine Ac3-Temperatur oder darüber und 1200 °C oder darunter,
Warmwalzen des Stahls mit einer kumulativen Walzreduktion von 40% oder mehr,
schnelles Abkühlen des Stahls von einer Ar3-Temperatur oder darüber auf eine niedrigere Temperatur, die sowohl auf 350 °C oder darunter als auch auf der Ar3-Temperatur oder darunter liegt, und
Anlassen des Stahls bei einer Temperatur im Bereich von 450 °C bis 700 °C.

3. Verfahren zum Herstellen eines dickwandigen, hochzähen, hochfesten Stahlblechs mit einer Dicke von 100 mm oder mehr, einer Dehngrenze von 620 MPa oder mehr, das in Masse-% umfasst:
0,08% bis 0,20% C,
0,40% oder weniger Si,
0,5% bis 5,0% Mn,
0,010 % oder weniger P,
0,0050% oder weniger S,
3,0% oder weniger Cr,
0,1% bis 5,0% Ni,
0,010% bis 0,080% Al,
0,0070% oder weniger N, sowie
0,0025% oder weniger O,
wenn die Formeln (1) und (2) gelten, optional
0,50 % oder weniger Cu,
1,50% oder weniger Mo,
0,400% oder weniger V,
0,100% oder weniger Nb,
0,005% bis 0,020% Ti,
0,0001% bis 0,0050% Mg,
0,01% bis 0,20% Ta,
0,005% bis 0,1% Zr,
0,001% bis 0,01% Y,
0,0030% oder weniger B,
0,0005% bis 0,0050% Ca, oder/und
0,0005% bis 0,0100% REM,
wobei ein Rest Fe und zufällige Verunreinigungen sind, und es eine Zähigkeit (vE-40) von 70 J oder mehr bei -40 °C in dem Oberflächenabschnitt des Grundmetalls aufweist: ${Ceq}^{IIW} = C + Mn / 6 + \left(Cu+Ni\right) / 15 + \left(Cr+Mo+V\right) / 5 \geq 0,65$ $\left({C}_{L}-C\right) / {C}_{L} \times 100 \geq 30$ wobei C_{L} durch die folgende Formel definiert wird: ${C}_{L} = 0,2 - \left(-0,1\times \left(0,2-Si\right)-0,03\times \left(1,1-Mn\right)-0,12\times \left(0,2-Cu\right)-0,11\times \left(3-Ni\right)+0,025\times \left(1,2-Cr\right)+0,1\times \left(0,5-Mo\right)+0,2\times \left(0,04-V\right)-0,05\times \left(0,06-Al\right)\right)$ wobei Element-Symbole in den Formeln den Gehalt (Masse-%) der jeweiligen Legierungsbestandteile angeben, und beim Nichtvorhandensein eines Elementes das Element-Symbol mit 0 angegeben wird, und
eine Querschnittsverminderung in einer Dickenrichtung bei der halben Blechdicke, die der prozentuale Anteil der Differenz zwischen der minimalen Querschnittsfläche, nachdem ein Zugversuch-Prüfkörper in Form eines Rundstabes, der den Abschnitt mit halber Dicke des Stahlblechs in der Dickenrichtung einschließt, in einem Zugversuch gebrochen war, und der ursprünglichen Querschnittsfläche relativ zu der ursprünglichen Querschnittsfläche ist, 40 % oder mehr beträgt,
wobei das Verfahren umfasst:
Erhitzen von Stahl auf 1200 °C bis 1350 °C,
Flachwalzen des Stahls mit einer kumulativen Walzreduktion von 40% oder mehr,
Erhitzen des Stahls auf eine Ac3-Temperatur oder darüber und 1200 °C oder darunter,
Warmwalzen des Stahls mit einer kumulativen Walzreduktion von 40% oder mehr, Abkühlen des Stahls,
erneutes Erhitzen des Stahls auf die Ac3-Temperatur oder darüber und 1050 °C oder darunter,
schnelles Abkühlen des Stahls von der Ac3-Temperatur oder darüber auf eine niedrigere Temperatur, die sowohl auf 350 °C oder darunter als auch auf einer Ar3-Temperatur oder darunter liegt, und
Anlassen des Stahls bei einer Temperatur im Bereich von 450 °C bis 700 °C.

4. Verfahren zum Herstellen eines dickwandigen, hochzähen, hochfesten Stahlblechs mit einer Dicke von 100 mm oder mehr, einer Dehngrenze von 620 MPa oder mehr, das in Masse-% umfasst:
0,08% bis 0,20% C,
0,40% oder weniger Si,
0,5% bis 5,0% Mn,
0,010 % oder weniger P,
0,0050% oder weniger S,
3,0% oder weniger Cr,
0,1% bis 5,0% Ni,
0,010% bis 0,080% Al,
0,0070% oder weniger N, sowie
0,0025% oder weniger O,
wenn die Formeln (1) und (2) gelten, optional
0,50 % oder weniger Cu,
1,50% oder weniger Mo,
0,400% oder weniger V,
0,100% oder weniger Nb,
0,005% bis 0,020% Ti,
0,0001% bis 0,0050% Mg,
0,01% bis 0,20% Ta,
0,005% bis 0,1% Zr,
0,001% bis 0,01% Y,
0,0030% oder weniger B,
0,0005% bis 0,0050% Ca, oder/und
0,0005% bis 0,0100% REM,
wobei ein Rest Fe und zufällige Verunreinigungen sind, und es eine Zähigkeit (vE-40) von 70 J oder mehr bei -40 °C in dem Oberflächenabschnitt des Grundmetalls aufweist: ${Ceq}^{IIW} = C + Mn / 6 + \left(Cu+Ni\right) / 15 + \left(Cr+Mo+V\right) / 5 \geq 0,65$ $\left({C}_{L}-C\right) / {C}_{L} \times 100 \geq 30$ wobei C_{L} durch die folgende Formel definiert wird: ${C}_{L} = 0,2 - \left(-0,1\times \left(0,2-Si\right)-0,03\times \left(1,1-Mn\right)-0,12\times \left(0,2-Cu\right)-0,11\times \left(3-Ni\right)+0,025\times \left(1,2-Cr\right)+0,1\times \left(0,5-Mo\right)+0,2\times \left(0,04-V\right)-0,05\times \left(0,06-Al\right)\right)$ wobei Element-Symbole in den Formeln den Gehalt (Masse-%) der jeweiligen Legierungsbestandteile angeben, und beim Nichtvorhandensein eines Elementes das Element-Symbol mit 0 angegeben wird, und wobei
eine Querschnittsverminderung in einer Dickenrichtung bei der halben Blechdicke, die der prozentuale Anteil der Differenz zwischen der minimalen Querschnittsfläche, nachdem ein Zugversuch-Prüfkörper in Form eines Rundstabes, der den Abschnitt mit halber Dicke des Stahlblechs in der Dickenrichtung einschließt, in einem Zugversuch gebrochen war, und der ursprünglichen Querschnittsfläche relativ zu der ursprünglichen Querschnittsfläche ist, 40 % oder mehr beträgt,
wobei das Verfahren umfasst:
Erhitzen von Stahl auf 1200 °C bis 1350 °C,
Flachwalzen des Stahls mit einer kumulativen Walzreduktion von 40% oder mehr,
Erhitzen des Stahls auf eine Ac3-Temperatur oder darüber und 1200 °C oder darunter,
Warmwalzen des Stahls mit einer kumulativen Walzreduktion von 40% oder mehr,
schnelles Abkühlen des Stahls von einer Ar3-Temperatur oder darüber auf eine niedrigere Temperatur, die sowohl auf 350 °C oder darunter als auch auf der Ar3-Temperatur oder darunter liegt, und
Anlassen des Stahls bei einer Temperatur im Bereich von 450 °C bis 700 °C.

## Revendications

1. Procédé de fabrication d'une plaque d'acier épaisse à haute résistance et haute ténacité ayant une épaisseur de 100 mm ou plus, une limite d'élasticité de 620 MPa ou plus et comprenant, sur une base de pourcentage massique,
C : 0,08 % à 0,20 %,
Si : 0,40 % ou moins,
Mn : 0,5 % à 5,0 %,
P : 0,010 % ou moins,
S : 0,0050 % ou moins,
Cr : 3,0 % ou moins,
Ni : 0,1 % à 5,0 %,
Al : 0,010% à 0,080%,
N : 0,0070 % ou moins et
O : 0,0025 % ou moins,
les formules (1) et (2) suivantes étant satisfaites, éventuellement au moins un élément parmi
Cu : 0,50 % ou moins,
Mo : 1,50 % ou moins,
V : 0,400 % ou moins,
Nb : 0,100 % ou moins,
Ti : 0,005 % à 0,020 %,
Mg : 0,0001 % à 0,0050 %,
Ta : 0,01 % à 0,20 %,
Zr : 0,005 % à 0,1 %,
Y : 0,001 % à 0,01 %,
B : 0,0030 % ou moins,
Ca : 0,0005 % à 0,0050 %, et
Terres rares : 0,0005 % à 0,0100 %,
le reste étant du Fe et des impuretés inévitables, et comprenant une ténacité (vE-40) de 70 J ou plus à -40 °C dans la partie de surface du métal de base : ${Ceq}^{IIW} = C + Mn / 6 + \left(Cu+Ni\right) / 15 + \left(Cr+Mo+V\right) / 5 \geq 0,65$ $\left({C}_{L}-C\right) / {C}_{L} \times 100 \geq 30$ C_{L} étant défini par la formule suivante : ${C}_{L} = 0,2 - \left(-0,1\times \left(0,2-Si\right)-0,03\times \left(1,1-Mn\right)-0,12\times \left(0,2-Cu\right)-0,11\times \left(3-Ni\right)+0,025\times \left(1,2-Cr\right)+0,1\times \left(0,5-Mo\right)+0,2\times \left(0,04-V\right)-0,05\times \left(0,06-Al\right)\right)$ où les symboles d'éléments dans les formules représentent les teneurs respectives (% en masse) des constituants d'alliage, et en l'absence d'un élément, le symbole de l'élément est représenté par 0, et où
une réduction de surface dans un sens épaisseur à la moitié de l'épaisseur de la plaque, qui est le pourcentage de la différence entre l'aire de section transversale minimum après la rupture d'une éprouvette en barreau à section ronde incluant la partie à la moitié de l'épaisseur de la plaque d'acier dans le sens épaisseur lors d'un essai de traction et l'aire de section transversale d'origine, rapportée à l'aire de section transversale d'origine, est de 40 % ou plus,
le procédé comprenant :
un chauffage de l'acier entre 1200 °C et 1350 °C,
un forgeage à chaud de l'acier avec un taux de réduction cumulé de 25 % ou plus,
un chauffage de l'acier à une température Ac3 ou plus et 1200 °C ou moins,
un laminage à chaud de l'acier avec un taux de réduction par laminage cumulé de 40 % ou plus,
un refroidissement naturel de l'acier,
un réchauffage de l'acier à la température Ac3 ou plus et 1050 °C ou moins,
un refroidissement rapide de l'acier depuis la température Ac3 ou plus jusqu'à une température inférieure qui est à la fois inférieure ou égale à 350 °C et inférieure ou égale à la température Ar3, et
un revenu de l'acier à une température dans la plage de 450 °C à 700 °C.

2. Procédé de fabrication d'une plaque d'acier épaisse à haute résistance et haute ténacité ayant une épaisseur de 100 mm ou plus, une limite d'élasticité de 620 MPa ou plus et comprenant, sur une base de pourcentage massique,
C : 0,08 % à 0,20 %,
Si : 0,40 % ou moins,
Mn : 0,5 % à 5,0 %,
P : 0,010 % ou moins,
S : 0,0050 % ou moins,
Cr : 3,0 % ou moins,
Ni : 0,1 % à 5,0 %,
Al : 0,010% à 0,080 %,
N : 0,0070 % ou moins et
O : 0,0025 % ou moins,
les formules (1) et (2) suivantes étant satisfaites, éventuellement au moins un élément parmi
Cu : 0,50 % ou moins,
Mo : 1,50 % ou moins,
V : 0,400 % ou moins,
Nb : 0,100 % ou moins,
Ti : 0,005 % à 0,020 %,
Mg : 0,0001 % à 0,0050 %,
Ta : 0,01 % à 0,20 %,
Zr : 0,005 % à 0,1 %,
Y : 0,001 % à 0,01 %,
B : 0,0030 % ou moins,
Ca : 0,0005 % à 0,0050 %, et
Terres rares : 0,0005 % à 0,0100 %,
le reste étant du Fe et des impuretés inévitables, et comprenant une ténacité (vE-40) de 70 J ou plus à -40 °C dans la partie de surface du métal de base : ${Ceq}^{IIW} = C + Mn / 6 + \left(Cu+Ni\right) / 15 + \left(Cr+Mo+V\right) / 5 \geq 0,65$ $\left({C}_{L}-C\right) / {C}_{L} \times 100 \geq 30$ C_{L} étant défini par la formule suivante : ${C}_{L} = 0,2 - \left(-0,1\times \left(0,2-Si\right)-0,03\times \left(1,1-Mn\right)-0,12\times \left(0,2-Cu\right)-0,11\times \left(3-Ni\right)+0,025\times \left(1,2-Cr\right)+0,1\times \left(0,5-Mo\right)+0,2\times \left(0,04-V\right)-0,05\times \left(0,06-Al\right)\right)$ où les symboles d'éléments dans les formules représentent les teneurs respectives (% en masse) des constituants d'alliage, et en l'absence d'un élément, le symbole de l'élément est représenté par 0, et où
une réduction de surface dans un sens épaisseur à la moitié de l'épaisseur de la plaque, qui est le pourcentage de la différence entre l'aire de section transversale minimum après la rupture d'une éprouvette en barreau à section ronde incluant la partie à la moitié de l'épaisseur de la plaque d'acier dans le sens épaisseur lors d'un essai de traction et l'aire de section transversale d'origine, rapportée à l'aire de section transversale d'origine, est de 40 % ou plus,
le procédé comprenant :
un chauffage de l'acier entre 1200 °C et 1350 °C,
un forgeage à chaud de l'acier avec un taux de réduction cumulé de 25 % ou plus,
un chauffage de l'acier à une température Ac3 ou plus et 1200 °C ou moins,
un laminage à chaud de l'acier avec un taux de réduction par laminage cumulé de 40 % ou plus,
un refroidissement rapide de l'acier depuis une température Ar3 ou plus jusqu'à une température inférieure qui est à la fois inférieure ou égale à 350 °C et inférieure ou égale à la température Ar3, et
un revenu de l'acier à une température dans la plage de 450 °C à 700 °C.

3. Procédé de fabrication d'une plaque d'acier épaisse à haute résistance et haute ténacité ayant une épaisseur de 100 mm ou plus, une limite d'élasticité de 620 MPa ou plus et comprenant, sur une base de pourcentage massique, C : 0,08 % à 0,20 %,
Si : 0,40 % ou moins,
Mn : 0,5 % à 5,0 %,
P : 0,010 % ou moins,
S : 0,0050 % ou moins,
Cr : 3,0 % ou moins,
Ni : 0,1 % à 5,0 %,
Al : 0,010% à 0,080 %,
N : 0,0070 % ou moins et
O : 0,0025 % ou moins,
les formules (1) et (2) suivantes étant satisfaites, éventuellement au moins un élément parmi
Cu : 0,50 % ou moins,
Mo : 1,50 % ou moins,
V : 0,400 % ou moins,
Nb : 0,100 % ou moins,
Ti : 0,005 % à 0,020 %,
Mg : 0,0001 % à 0,0050 %,
Ta : 0,01 % à 0,20 %,
Zr : 0,005 % à 0,1 %,
Y : 0,001 % à 0,01 %,
B : 0,0030 % ou moins,
Ca : 0,0005 % à 0,0050 %, et
Terres rares : 0,0005 % à 0,0100 %,
le reste étant du Fe et des impuretés inévitables, et comprenant une ténacité (vE-40) de 70 J ou plus à -40 °C dans la partie de surface du métal de base : ${Ceq}^{IIW} = C + Mn / 6 + \left(Cu+Ni\right) / 15 + \left(Cr+Mo+V\right) / 5 \geq 0,65$ $\left({C}_{L}-C\right) / {C}_{L} \times 100 \geq 30$ C_{L} étant défini par la formule suivante : ${C}_{L} = 0,2 - \left(-0,1\times \left(0,2-Si\right)-0,03\times \left(1,1-Mn\right)-0,12\times \left(0,2-Cu\right)-0,11\times \left(3-Ni\right)+0,025\times \left(1,2-Cr\right)+0,1\times \left(0,5-Mo\right)+0,2\times \left(0,04-V\right)-0,05\times \left(0,06-Al\right)\right)$ où les symboles d'éléments dans les formules représentent les teneurs respectives (% en masse) des constituants d'alliage, et en l'absence d'un élément, le symbole de l'élément est représenté par 0, et où
une réduction de surface dans un sens épaisseur à la moitié de l'épaisseur de la plaque, qui est le pourcentage de la différence entre l'aire de section transversale minimum après la rupture d'une éprouvette en barreau à section ronde incluant la partie à la moitié de l'épaisseur de la plaque d'acier dans le sens épaisseur lors d'un essai de traction et l'aire de section transversale d'origine, rapportée à l'aire de section transversale d'origine, est de 40 % ou plus,
le procédé comprenant :
un chauffage de l'acier entre 1200 °C et 1350 °C,
un dégrossissage de l'acier avec un taux de réduction par laminage cumulé de 40 % ou plus,
un chauffage de l'acier à une température Ac3 ou plus et 1200 °C ou moins,
un laminage à chaud de l'acier avec un taux de réduction par laminage cumulé de 40 % ou plus, un refroidissement naturel de l'acier,
un réchauffage de l'acier à la température Ac3 ou plus et 1050 °C ou moins,
un refroidissement rapide de l'acier depuis la température Ac3 ou plus jusqu'à une température inférieure qui est à la fois inférieure ou égale à 350 °C et inférieure ou égale à une température Ar3, et
un revenu de l'acier à une température dans la plage de 450 °C à 700 °C.

4. Procédé de fabrication d'une plaque d'acier épaisse à haute résistance et haute ténacité ayant une épaisseur de 100 mm ou plus, une limite d'élasticité de 620 MPa ou plus et comprenant, sur une base de pourcentage massique,
C : 0,08 % à 0,20 %,
Si : 0,40 % ou moins,
Mn : 0,5 % à 5,0 %,
P : 0,010 % ou moins,
S : 0,0050 % ou moins,
Cr : 3,0 % ou moins,
Ni : 0,1 % à 5,0 %,
Al : 0,010% à 0,080 %,
N : 0,0070 % ou moins et
O : 0,0025 % ou moins,
les formules (1) et (2) suivantes étant satisfaites, éventuellement au moins un élément parmi
Cu : 0,50 % ou moins,
Mo : 1,50 % ou moins,
V : 0,400 % ou moins,
Nb : 0,100 % ou moins,
Ti : 0,005 % à 0,020 %,
Mg : 0,0001 % à 0,0050 %,
Ta : 0,01 % à 0,20 %,
Zr : 0,005 % à 0,1 %,
Y : 0,001 % à 0,01 %,
B : 0,0030 % ou moins,
Ca : 0,0005 % à 0,0050 %, et
Terres rares : 0,0005 % à 0,0100 %,
le reste étant du Fe et des impuretés inévitables, et comprenant une ténacité (vE-40) de 70 J ou plus à -40 °C dans la partie de surface du métal de base : ${Ceq}^{IIW} = C + Mn / 6 + \left(Cu+Ni\right) / 15 + \left(Cr+Mo+V\right) / 5 \geq 0,65$ $\left({C}_{L}-C\right) / {C}_{L} \times 100 \geq 30$ C_{L} étant défini par la formule suivante : ${C}_{L} = 0,2 - \left(-0,1\times \left(0,2-Si\right)-0,03\times \left(1,1-Mn\right)-0,12\times \left(0,2-Cu\right)-0,11\times \left(3-Ni\right)+0,025\times \left(1,2-Cr\right)+0,1\times \left(0,5-Mo\right)+0,2\times \left(0,04-V\right)-0,05\times \left(0,06-Al\right)\right)$ où les symboles d'éléments dans les formules représentent les teneurs respectives (% en masse) des constituants d'alliage, et en l'absence d'un élément, le symbole de l'élément est représenté par 0, et où
une réduction de surface dans un sens épaisseur à la moitié de l'épaisseur de la plaque, qui est le pourcentage de la différence entre l'aire de section transversale minimum après la rupture d'une éprouvette en barreau à section ronde incluant la partie à la moitié de l'épaisseur de la plaque d'acier dans le sens épaisseur lors d'un essai de traction et l'aire de section transversale d'origine, rapportée à l'aire de section transversale d'origine, est de 40 % ou plus,
le procédé comprenant :
un chauffage de l'acier entre 1200 °C et 1350 °C,
un dégrossissage de l'acier avec un taux de réduction par laminage cumulé de 40 % ou plus,
un chauffage de l'acier à une température Ac3 ou plus et 1200 °C ou moins,
un laminage à chaud de l'acier avec un taux de réduction par laminage cumulé de 40 % ou plus,
un refroidissement rapide de l'acier depuis une température Ar3 ou plus jusqu'à une température inférieure qui est à la fois inférieure ou égale à 350 °C et inférieure ou égale à la température Ar3, et
un revenu de l'acier à une température dans la plage de 450 °C à 700 °C.
